

# UNITED STATES PATENT OFFICE.

WILLIAM D. COOLIDGE, OF SCHENECTADY, NEW YORK, ASSIGNEE TO GENERAL ELECTRIC COMPANY, A CORPORATION OF NEW YORK.

## METAL FILAMENT.

1,026,382.

Specification of Letters Patent. Patented May 14, 1912.

No Drawing.

Application filed May 9, 1906. Serial No. 316,005.

To all whom it may concern:

Be it known that I, WILLIAM D. COOLIDGE, a citizen of the United States, residing at Schenectady, county of Schenectady, State 5 of New York, have invented certain new and useful Improvements in Metal Filaments, of which the following is a specification.

This invention pertains to the art of in- 10 candescent conductors such as are used in electric lamps and other apparatus.

Many of the more refractory metals and 15 elements have been suggested for use in incandescent lamps and in other apparatus where a conducting body is raised to an ex- 20 ceedingly high temperature. Some of these refractory elements are, however, very difficult to shape into filaments because of the difficulty of obtaining them in a wire or other slender conductor. Tungsten is an 25 example of this class of elements. It is ordinarily obtained as a fine powder, the particles of which do not readily cohere and cannot be agglomerated into a coherent product without some special treatment.

According to this invention, a refractory material such as tungsten is incorporated in a metallic body, such as a ductile alloy, and the mixture so formed is shaped into a 30 filament in any suitable way, and is then treated to drive out all components except the refractory material, the latter remaining behind as a coherent product. I may use various refractory metals or elements such 35 as tungsten, molybdenum, boron, zirconium, titanium, thorium, tantalum, etc., and I may bind the separate particles of the powder together with various ductile alloys or metals.

I will explain the process as applied to 40 tungsten using a bismuth cadmium alloy as a binder, and it is to be understood that the same general process is applicable to other refractory metals, elements, and compounds, and that other binders may be used.

45 I purify the tungsten to make sure that no impurities such as carbon are present. I may also subject it to a special treatment to insure a very finely divided powder. This special process of pulverizing or sub- 50 dividing may consist in forming a colloidal solution in one of many well known ways, and then driving off the liquid of the solution to leave behind fine particles of tung- 55 sten. The colloid may be produced by form- ing an arc between tungsten electrodes under

a liquid, or may be made chemically and purified by dialysis.

Still another method of insuring a fine powder consists in mixing the original powder with water, or other suitable liquid and 60 allowing the powder to precipitate out. The fraction which comes out last is, of course, finer than the part first precipitated. One of the advantages of having an exceedingly 65 fine powder arises from the ease with which such a powder may be incorporated in another metal and squirted through a very fine die to produce filaments of small cross-section. Another advantage is the smooth 70 surface which the filament has when very fine powder is used.

I next produce an alloy of cadmium and bismuth by melting these two metals together over a gas flame or other source of heat. The proportions of the two components may vary, but good results may be obtained by using 208 parts by weight of bismuth and 112 by weight of cadmium, thus producing an alloy of proper proportions to satisfy the formula BiCd. I next heat some 80

of this alloy to the plastic condition and rub into it the tungsten powder above mentioned. The exact proportion of tungsten to be added may vary between considerable limits; but if 53 per cent. by weight is used, 85 the product can be readily manipulated and is otherwise satisfactory. This operation may be carried out by merely adding the tungsten to the alloy in a chemist's mortar and rubbing the mixture with a pestle until 90 it is homogeneous. I do not at present believe that the tungsten combines with the alloy, but think it is merely suspended and held together by the alloy acting as a binding agent. The tungsten may be added to 95

the alloy and mixed therewith in the open air and the melting point of the alloy, about 144° centigrade, is not sufficiently high to produce any oxidation of the tungsten. If I use some other binding metal or alloy having a melting point higher than that at which tungsten oxidizes in the open air, then I find it desirable to perform this mixing operation in an inert atmosphere or in a vacuum. The mixture of tungsten and metallic binding material above described is next shaped into wires or filaments by squirting through a die. I find that I can squirt filaments as fine as would probably ever be desired in electric lamps, or I can 110

squirt filaments of moderate size and draw them down through suitable draw plates to the desired diameter. These filaments are ductile, may be readily coiled or bent without breaking, and are comparatively strong under tensile stress. I find it desirable to warm the material somewhat in performing the squirting operation. The next step in my process consists in treating these filaments to drive out all components except the tungsten or such other refractory metal or metals as may have been used; or at least to drive out all the easily vaporizable materials. This may be conveniently done by mounting the filaments in vacuum globes or in an inert atmosphere and passing current through the filaments to heat them. The easily vaporizable components, such as bismuth and cadmium, come out very easily,— and, so far as I have determined, very completely,—and leave behind a coherent metallic product capable of operating at an exceedingly high temperature and consequently at good light efficiency. If desired, the distillation of the cadmium-bismuth alloy may be effected in a few moments, but I may heat for a much longer time to prevent a sudden rush of vapors within the filament. After distillation is complete, I may heat the filament with current to a very high temperature to sinter together the particles of tung-

sten or other refractory residue and improve the filament as a light giving conductor. The final product is a strong, uniform conductor, homogeneous in composition and very refractory. 35

In certain of the claims appended hereto I have used the word "metal", and I desire it to be understood that this term is used in the popular sense of either a metallic element, an alloy, or a metallic mixture. 40

What I claim as new and desire to secure by Letters Patent of the United States, is:

1. The composition consisting of a cadmium - bismuth alloy containing metallic 45 tungsten.

2. The composition consisting of a bismuth alloy containing refractory metal.

3. The composition consisting of a cadmium-bismuth alloy containing finely di- 50 vided refractory metal.

4. A conductive pliant wire consisting of fine particles held together by a cadmium-bismuth alloy adapted to be converted into a refractory incandescent body by suitable 55 heat treatment.

In witness whereof, I have hereunto set my hand this 8th day of May, 1906.

WILLIAM D. COOLIDGE.

Witnesses:

BENJAMIN B. HULL,  
HELEN ORFORD.